

(No Model.)

F. SEDGWICK.

METHOD OF TEMPERING SPIRAL SPRINGS.

No. 401,721.

Patented Apr. 16, 1889.



FIG. 1.



FIG. 2.

Witnesses:

J. B. Halpenny  
David Stearns.

Inventor:

Frederick Sedgwick  
By G. L. Fletcher  
his Atty.

# UNITED STATES PATENT OFFICE.

FREDERICK SEDGWICK, OF CHICAGO, ILLINOIS, ASSIGNOR TO THE AMERICAN SPRING COMPANY, OF ILLINOIS.

## METHOD OF TEMPERING SPIRAL SPRINGS.

SPECIFICATION forming part of Letters Patent No. 401,721, dated April 16, 1889.

Application filed December 2, 1887. Serial No. 256,741. (No model.)

*To all whom it may concern:*

Be it known that I, FREDERICK SEDGWICK, of Chicago, in the county of Cook and State of Illinois, have invented a certain new, useful, and Improved Method of Tempering Spiral Springs, of which the following is a description, reference being had to the accompanying drawings, forming a part of this specification, in which like letters of reference in the 10 different figures designate like parts.

Heretofore in the tempering of spiral springs it has been customary to wind the tempered wire when cold upon a former of the desired shape. This method has been found 15 to be objectionable, in that the molecules of the metal upon the outside of the coil have been strained or stretched, while those upon the inside have been unduly compressed, thus greatly weakening and impairing the value 20 of the spring. To meet this difficulty and to restore the "nature" to the spring, it has been customary, after forming the same, as above stated, to submit it in an oven or muffle to a heat of about 600° Fahrenheit, or there- 25 about, for a sufficient time to cause the molecules of the metal to assume their normal relations. While this strengthens, and in a measure imparts new life to the spring, yet it does not accomplish the desired result. More- 30 over, the reheating of the metal is injurious in itself and should be avoided, if possible.

The object of my invention is to provide a method whereby a steel wire or ribbon may be formed into a spiral or coil while the steel 35 is heated to a red heat and is soft or ductile, and while in this condition and form chilled or tempered, the whole being done simultaneously and in one operation, and serving to produce a hot-set spring, thus obviating the 40 defects above described, all of which is hereinafter described, claimed, and shown in the drawings, in which—

Figure 1 is a side view of a reel, mandrel, cooling-bath, and dynamo-electric machine, 45 the whole constituting my improved apparatus for coiling and tempering springs, and Fig. 2 is a plan view thereof.

Referring to the drawings, A represents a base or support, upon which is loosely placed 50 an oblong vessel, B, adapted to slide across said base in guides b b. Said vessel is, by

preference, wholly or partially filled with mercury, as shown in Fig. 1, for the purposes hereinafter stated.

C is a mandrel or former mounted in bearings c c, Fig. 2, so as to be readily removed therefrom.

D is a shaft loosely mounted in a bearing, d, secured to the trough B. Upon the inner end of said shaft is a gear-wheel, D', which engages with a gear, C', rigidly attached to the mandrel C.

D<sup>2</sup> is a crank by which the shaft is rotated, and D<sup>3</sup> is a worm-gear, which engages with a rack, E, attached, by means of standards E', to the base A.

F is a reel, and G is a wire extending therefrom to the mandrel C, to which one end is attached, as shown in Fig. 2.

H is a standard attached rigidly to the base 70 A, and to which in turn is secured, and preferably insulated therefrom, a spring-clamp, J, and binding-post J'.

K is a dynamo, one pole of which is connected with the binding-post J' by means of 75 a wire, k, and the other, by a wire, k', to a binding-post, B', secured to the trough B and having a metal strip, B<sup>2</sup>, which extends into the mercury of said trough.

The wire G passes from the reel through 80 the clamp J, and thus that portion between said clamp and the mandrel C serves to complete the electric circuit with the wires k k', said mandrel thus forming one pole of the circuit with the wire to be tempered. As 85 soon as the end of the wire is attached to the mandrel and the electric circuit closed, the wire between the mandrel and clamp J becomes heated, when the crank D<sup>2</sup> is turned, thus winding the heated wire upon the man- 90 drel. The mandrel being cold, by virtue of its continual contact with the mercury, serves to suddenly chill the wire and impart thereto a

spring-temper, provided the strength of the electric current is so regulated as to cause the 95 proper degree of heat, which is indicated by a dull or low-red color. The cooling-bath into which the wire is wound also aids to chill said wire. As the mandrel is revolved, it is also moved longitudinally by means of the worm 100 D<sup>3</sup> and rack E, so as to impart the desired pitch to the spiral. Upon reaching the end

of the mandrel the electric circuit is broken and the spring removed, when the operation may be repeated.

While I prefer to revolve the mandrel in a bath of mercury, it is obvious that any other cooling medium may be employed which will not tend to impair the electric contact of the wire with the mandrel. To this end the mandrel may be made hollow, and water may be made to circulate therein. In the latter event the strip B<sup>2</sup>, which might form a "brush," should be brought into direct contact with the mandrel, so that the latter may form one pole of the electric circuit.

I am aware that it is old in the manufacture of coiled springs to successively and continuously heat, harden, and temper, and then coil the wire into spring form while it yet retains its tempering-heat, and I make no claim to such method; but form the coil while the metal is in such a ductile condition as to require chilling to give it a temper, as distinguished from coiling after a temper has been imparted to it. To accomplish this result, it is obvious that the wire should be heated to a red heat as nearly as possible to its point of contact with the mandrel. This is best effected by employing electric heat and causing

the mandrel to form one electrode. In coiling small wire, which only retains its heat for an instant, the importance of this feature is manifest. The result of this method is a hot-set spring bent or formed while the metal is soft or ductile.

One advantage of said method, aside from its cheapness, is, that the wire, being bent upon the mandrel while hot and chilled thereon, will retain its strength and resiliency to the utmost, and will require no further treatment than the mere drawing of the temper in any well-known way, to make a perfect spring.

Having thus described my invention, I claim—

The method, substantially as herein shown and described, in the manufacture of coiled springs, which consists in simultaneously heating the steel wire or strip to redness or a ductile condition, winding and chilling the same upon a former or mandrel, and afterward drawing the temper in any well-known way.

FREDERICK SEDGWICK.

Witnesses:

D. H. FLETCHER,  
J. B. HALPENNY.